

# UNITED STATES PATENT OFFICE.

HÈLÈNE RACHEL HIRSCHLER, OF PARIS, FRANCE, ASSIGNOR TO J. HAYEM & CO., OF SAME PLACE.

## IMPREGNATING FABRICS WITH ANTISEPTIC SALTS.

SPECIFICATION forming part of Letters Patent No. 564,928, dated July 28, 1896.

Application filed April 6, 1895. Serial No. 544,803. (No specimens.) Patented in France November 26, 1893, No. 234,161; in England April 4, 1894, No. 6,747, and in Germany April 29, 1894, No. 77,880.

To all whom it may concern:

Be it known that I, HÈLÈNE RACHEL HIRSCHLER, of Paris, in the Republic of France, have invented an Improved Mode of 5 Rendering Fabrics Impervious to Infection, (for which I have obtained a patent in France, dated November 26, 1893, No. 234,161; in Germany, dated April 29, 1894, No. 77,880, and in Great Britain, dated April 4, 1894, No. 6,747,) 10 of which the following is a specification.

The object of this invention is to render garments, fabrics, or tissues impervious to infection; and the invention consists in impregnating the garments, fabrics, or tissues with 15 a substance which is antiseptic and an absolutely inoffensive microbicide and without odor, and which will allow of the garments or other fabrics being washed continuously without losing their antiseptic properties.

Up to this date no one has succeeded in 20 fixing an antiseptic substance in a fabric, and especially so with respect to flannel, because no one has been able to find an antiseptic which can be rendered insoluble, and 25 becomes, so to speak, incorporated in the fibers of the fabric.

In carrying out this invention the fabric is first treated with a lukewarm solution of 30 a metallic salt, which acts as a kind of mordant to prepare the fabric to take up an antiseptic in solution, and also forms a base or support to carry the antiseptic, and it further renders the antiseptic non-volatile and permanent, in the sense that it will permit of the 35 fabric being washed without losing its properties, and, secondly, the fabric is dipped in an antiseptic solution.

The metallic salts used is one the oxid of 40 which does not possess toxical properties, and at the same time is capable of forming 45 an insoluble combination, intimately fixed in the fiber when the fabric is submitted to immersion in a solution of an organic acid of the aromatic series constituting an antiseptic, and such metallic salt may be a soluble salt of bismuth or tin or aluminium.

The antiseptic which is used is salicylic acid or one of its homologues or combinations, such as bromo or iodo salicylic acid or 50 their soluble salts, or it may be benzoic or

cresotinic acids or their combinations. In a word, any other antiseptic acid or salt capable of forming on the fiber an insoluble salt of the metal used may be employed.

The first bath containing the metallic salt 55 to form the mordant base or support is prepared from the following ingredients, the quantities of which are calculated for the treatment of about ten kilograms of fabric: One hundred and twenty-five to one hundred 60 and fifty grams nitrate of bismuth or one hundred and twenty-five grams chlorid or bichlorid of tin dissolved in two hundred to two hundred and fifty grams crystallizable acetic acid, warm. After the fabric has 65 remained in the bath about half an hour, it will be found that it has absorbed all the metallic oxid contained therein. The fabric is then removed, and after being rinsed is passed through the second bath, composed of 70 from sixty to one hundred grams of salicylic acid or its homologues.

In case the mordanting bath is tin a saline combination, such as salicylate of soda, will 75 be found to answer better than salicylic acid alone. The effect which takes place on bringing the salicylic acid into the presence of the metallic salt is to produce an insoluble salicylate of bismuth or tin, as the case may be, with which the fabric becomes impregnated. 80

If the mordanting bath is composed of a salt of aluminium, the acetate is preferably employed. Then the second bath will be composed of benzoic acid or an alkaline benzoate, the substance thus produced being an 85 insoluble benzoate of aluminium, with which the fabric is impregnated.

A bath may be formed from bromo or iodo salicylic acid, or, it may be, cresotinic acid, or, as before stated, any other antiseptic acid 90 or salt capable of forming, with the metal used for the first bath, an insoluble metallic salt on the fiber of the fabric; or I may employ a combination of two antiseptics—viz., salicylic acid and tannic acid, (commercial 95 tannin,) and these will be found to possess great fixity and resistance to bleaching solutions of various kinds.

In carrying out this part of my invention the fabric is first dipped in a bath of a salt 100

of tin, for example, chlorid or oxychlorid of tin, having six per cent. of the weight of the fabric in protochlorid, dissolved by means of hydrochloric acid, which is employed in a sufficient quantity to obtain a complete solution. The fabric is then removed, and after rinsing is passed through a second bath containing in tannic acid two per cent. of the weight of the fabric under treatment. The fabric is again removed and rinsed and finally passed through a third bath, containing a solution of three per cent. of salicylic acid and Solvay's soda in the proportion of an eighth part by weight of the acid used.

15 The fabric should be left in each bath about half an hour. The temperature of the tin bath and of the salicylic-acid bath should be raised to boiling-point, the temperature of the second bath being, preferably, that of 20 warm water.

Although I have mentioned garments and fabrics or tissues only, the invention is applicable to vegetable or animal fibers generally, such as used, for example, for mattresses 25 or bedding, or stuffing for articles of furniture,

or feathers used for pillows, or to down for quilts, or for any other materials or substances which are liable to become infected with microbes or germs of diseases, all of which, for the purposes of this invention, I 30 include under the word "fabrics."

Having now particularly described and ascertained the nature of my said invention and in what manner the same is to be performed, I declare that what I claim is—

35 The mode of rendering fabrics impervious to infection as herein described, consisting in impregnating the fabric with a solution of a metallic salt, such as chlorid of tin, and subsequently immersing the so-impregnated fabric in a solution of an organic acid, such as salicylic acid, as set forth.

In testimony whereof I have signed my name to this specification in the presence of two subscribing witnesses.

HIÉLÈNE RACHEL HIRSCHLER.

Witnesses:

LÉON CRAMKENS,  
CLYDE SHROPSHIRE.